

May 3, 1938.

E. W. SMITH

2,116,367

APPARATUS FOR TREATING METALS

Filed Oct. 17, 1935

2 Sheets-Sheet 1



FIG. 1



FIG. 2



FIG. 3

INVENTOR.

EDWARD W. SMITH

BY

Ezekiel Mef

ATTORNEY.

May 3, 1938.

E. W. SMITH

2,116,367

APPARATUS FOR TREATING METALS

Filed Oct. 17, 1935

2 Sheets-Sheet 2



FIG. 4



FIG. 5

INVENTOR.

EDWARD W. SMITH

BY

*Eugene Wolf*

ATTORNEY.

## UNITED STATES PATENT OFFICE

2,116,367

## APPARATUS FOR TREATING METALS

Edward W. Smith, Melrose, Mass., assignor to  
Submarine Signal Company, Boston, Mass., a  
corporation of Maine

Application October 17, 1935, Serial No. 45,442

11 Claims. (Cl. 22—57)

The present invention relates to a process and apparatus for the treatment of metals. In particular the present invention relates to a process and apparatus for treating molten metals to obtain a fine grain structure in the solidified metal.

In the manufacture of steel and other metals or alloys it is often highly desirable to obtain a solidification of the metal with a very fine grain structure. This, for example, is of great importance in the manufacture of stainless steel. It is also of great importance in the production of cast zinc ingots which are used as the primary source of metals for rolling out the zinc plates used for etching in the printing industry.

According to the present invention the molten metal after being poured into a mold or crucible is vibrated while it is cooling. When molten metal is poured into a mold and allowed to cool, the cooling is accomplished by a crystal formation which begins on the inside surface of the mold and develops towards the center. Under the ordinary quiet cooling conditions a series of relatively large crystals are thus produced and the ingot tends to be relatively weak at the center. According to my invention I bring about a continuous relative movement of vibration of the molten liquid with respect to its container. The vibration may be obtained by oscillating the mold or crucible preferably about its vertical axis or along its vertical axis. With the crucible in torsional vibration about its vertical axis the molten metal will tend to remain quiet, the crucible alone moving.

Under these conditions any crystals which form will have to form on a surface which is moving with respect to the molten metal from which they must come so that there is at all times a shearing action on any crystals which form which tends to break them up and thereby provides a finer structure in the solidified mass. The relative motion between the molten metal and the crucible takes place continuously until the metal is entirely solidified since each layer which cools on the inside of the crucible will in effect provide a new surface for the growth of each new layer of crystals. Crystal growth under these conditions results in a more homogeneous mass of small crystals rather than in a series of relatively large crystals as is the case where no vibration is applied.

It will be evident that vibrations may be applied in other modes than by the torsional vibration of the crucible provided relative motion between the crucible and the molten metal is always obtained. For example, instead of torsionally vi-

brating the crucible it may be vibrated vertically along its vertical axis.

The method of vibrating the crucible torsionally is preferable because a smaller absolute velocity of the crucible is required than with vertical vibrations. With this torsional method of vibration the shearing action between the molten metal and the crucible or solidified metal takes place in a direction perpendicular to the direction of cooling at all times between planes of metal of different temperatures.

An important point to be observed is that relative motion must be obtained between the fluid metal and the crucible or solidified metal to provide the necessary shearing action. The vibration must thus have a sufficient velocity to bring about this result. In case the mold is to be vibrated vertically, precautions must be taken to see that the frequency and amplitude of vertical motion are such as to ensure a velocity of motion of the crucible which is greater than that which would be attained by the molten metal under the influence of gravity alone.

The vibration of the cooling crucible or mold with respect to the molten liquid may be carried out with any suitable vibratory apparatus. However, I prefer to use a vibrating system which in itself is resonant at the desired frequency.

Suitable forms of vibrating apparatus are shown in the accompanying drawings in which Fig. 1 is a sectional elevation of an apparatus for torsionally vibrating a mold or crucible; Fig. 2 is a horizontal section on the line A—A of the apparatus shown in Fig. 1; Fig. 3 is a horizontal section on the line B—B on the device shown in Fig. 1; Fig. 4 is a vertical section of an arrangement for vibrating a crucible or mold in a vertical direction; and Fig. 5 is a modification of Fig. 4.

The mold or crucible 1 in Fig. 1 is preferably circular in cross section and cylindrical or conical in shape. It is secured to a small table 2 by locking screws 3 which hold the crucible securely to the table 2. Suitable heat-insulating material 4 separates the table from the frame 5. The latter is supported on a platform 6 by means of roller or ball bearings 7 and itself supports and is rigidly secured to the field pieces 27 of an oscillatory motor. The platform 6 is supported upon a base 8 by ball bearings 10. A shaft 11 is secured to the platform 6 and its lower end projects into a well 12 in the base 8. Ball bearings 13 provided in the well 12 and ball bearings 14 suitably mounted in the upper part of the frame 5 serve to keep the shaft 11 in a vertical

position. Rigidly secured to the shaft 11 are an armature 15 and a spring 16. The spring 16 is spiral in shape and is best seen in Fig. 3. It will be seen that one end of the spring is secured by rivets 18 to a collar or flange 17 on the shaft 11 while the other end of the spring is secured by rivet 19 to the frame 5. The arrangement of the armature and the pole pieces are shown in Fig. 2.

10 It will be noted that there are four pole pieces 24, 25, 26 and 27 which are formed by laminations held together by the bolts 8. Each of the pole pieces is surrounded by a coil 28 whereby the magnetic circuit is energized. The armature 15 is separated from the poles by an airgap of suitable dimensions and may conveniently be provided with two windings which are axially disposed around the armature and which are at right angles to one another. It will be clear 15 from Fig. 2 that if the coils 28 on the poles are properly connected together, the direction of flow of the flux can be made to be from poles 24 and 27 to poles 25 and 26, respectively, with a given direction of flow of the current through 20 the windings on the armature. It will also be clear that when current flows through the portion 24' of the windings nearest to pole 24 in a direction perpendicular to and towards the plane of the paper, it will be flowing in a direction perpendicular to and away from the plane of the paper in that portion of the winding which is 25 nearest pole 26; thus when the direction of the flow of flux in poles 24 and 27 is through the armature 15 and toward poles 25 and 26, the 30 passage of current in the direction away from the plane of the paper in the portion of the winding designated as 26' will tend to produce a counter-clockwise rotation of the armature 15. A similar tendency to counter-clockwise rotation 35 will be brought about by the currents in the other windings of the armature.

If the armature coils are properly connected in series with the coils on the poles, the flow of alternating current through the system will always tend to produce a counter-clockwise rotation 40 of the armature. This force will be such as to tend to wind up the spring 16. When the alternating current commences to decrease, the restoring force of the spring will rotate the armature in a clockwise direction until the alternating current passes through zero and again increases 45 in the reverse direction. This again brings about a counter-clockwise rotation of the armature in winding up the spring. This action results in an oscillatory rotation of the armature and of the frame 15.

The amplitude of this oscillatory rotation or torsional vibration will be a maximum at the resonance frequency of the system which is dependent upon the relative masses of the two major elements of the system and upon the strength of the spring. The two major masses of the system are obviously the armature and platform member 6, on the one hand, and the crucible and its supporting frame 5 carrying the pole pieces, on the other hand. The amplitude of the torsional vibration at resonance is proportional to the magnitude of the current in the windings and if the two masses are equal, they both will have the same amplitude of oscillation. Furthermore, the frequency of the alternating current which must be supplied to the system to obtain resonance must be one-half of the natural resonant frequency of the system.

75 In this manner the crucible 1 is vibrated tor-

sionally about its vertical axis. Since the inertia of the molten metal within the crucible keeps it substantially at rest, a relative motion is obtained between the walls of the crucible and the molten metal.

Instead of vibrating the crucible torsionally, it may be vibrated in the direction of its vertical axis. For this purpose the arrangement shown in Fig. 4 may conveniently be employed. Here the crucible 31 is preferably of a square or rectangular shape rather than of the conical shape of the crucible shown in Fig. 1, although a cylindrical crucible may also be used. The crucible 31 rests upon a table 32 which is insulated by thermal insulating material 34 from the supporting frame 35. The crucible 31 is secured by means of the screws 33 to the table 32 and the latter, in turn, is secured to the frame 35 by means of the bolts 36. The frame 35 is supported by the spring 37 upon the floor 38 of the building. The springs 37 are so designed that their fundamental and harmonic natural frequencies are different from the operating frequency of the system. This frequency difference is preferably about 20%.

Attached to the frame 35 are pole pieces 39 and a yoke member 40 by means of the bolts 41. These members form the electromagnetic field of an oscillator whose armature is shown at 42. The armature is fixed to the shaft 43 which, in turn, is rigidly connected to the mass 44 having an upwardly extending flange 45 which just fits within and serves as a guide for the downwardly extending flange 46 which is attached to or forms a part of the frame 35.

The mass comprising the magnetic field system which carries the crucible 31 is coupled by means of the spring 47 to the mass 44 to which the armature is connected. The ends of the armature shaft 43 are fitted to slide within the 40 bearings 48 and 49. When the magnets 39 are supplied with alternating current, they will tend to move by magnetic attraction toward and away from the armature 42. In this manner the crucible 31 is vibrated vertically.

The resonant frequency of the system is determined by the relations between the two masses and the stiffness of the coupling spring 47. The maximum amplitude of vibration will be obtained when the alternating current supplied to the 50 magnets 39 has a frequency equal to one-half the natural frequency of the system. If the two masses of the system be made equal, both will have the same amplitude. By increasing the size of the mass 44, the amplitude of the other mass 55 which includes the crucible 31 may be increased, or vice versa.

A modified form of a vertically vibrating system is shown in Fig. 5. In this figure the crucible carrying frame 35 is rigidly fixed to the 60 armature 42 which is supported directly upon the spring 47. The latter, in turn, is fixed to the frame 50 which in this case carries the field magnets 39 and is rigidly fastened to the floor of the building or other support 38. The vibratory system in this case comprises the substantially infinite mass 38 which is coupled through the spring 47 to the mass member comprising the armature and the crucible. This arrangement is somewhat simpler than that shown in 70 Fig. 4, but it must be mounted upon a very firm base 38 in order to avoid any transfer of energy thereto.

While I have described an apparatus for torsionally and vertically vibrating the mold or 75

5 crucible containing the molten metal, it will be evident to those skilled in the art that modifications of the arrangements shown may be made without departing from the spirit of the invention, and, furthermore, it will also be evident that if desired the mold may be vibrated in a horizontal direction and that the apparatus shown may readily be modified for this purpose.

Having now described my invention, I claim:

10 1. Apparatus for imparting rotational oscillations to a mold for molten metal comprising a mass member rigidly fixed to said mold, electromagnetic field elements secured to said mass member, a base, means for rotatably mounting said mold and connected elements upon said base, a second mass member rotatably mounted on said base, a shaft secured to said second mass member, an electromagnetic armature secured to said shaft and adapted to cooperate with said field 15 magnets and spring means mechanically coupling said armature shaft and said first mass member.

20 2. Apparatus for rotationally oscillating a container for molten metal comprising, in combination, therewith a table structure for supporting the same adapted to permit it to oscillate freely, an independent mass member having a magnitude at least substantially equal to the mass of said container when filled plus associated elements, means for supporting said mass member so that it is free to oscillate with respect to said container and resilient means adapted to provide between said container and said mass element a restoring force sufficient to make the system 25 resonant at the desired frequency of oscillation.

30 3. Apparatus for rotationally oscillating molten metal including a container therefor, means for supporting the same comprising a base member, a supporting frame to which said container can be fastened, bearing means for supporting said frame on said base so as to be free to oscillate, an independent mass element having a magnitude of substantially the same order as the mass of said container when filled plus the elements associated therewith, bearing means for supporting said mass element upon said base so as to be free to oscillate independently of said container supporting frame, resilient means coupling said mass element and said frame and adapted to provide a restoring force sufficient to make the natural 35 frequency of the system equal to the desired vibration frequency and means for imparting rotational vibration impulses to said system.

40 4. Apparatus for rotationally oscillating a mold for molten metal comprising an oscillatory electric motor having armature and field elements, a stationary base member, means for supporting both said elements upon said base so as to be freely oscillatable with respect to the base and to each other, means for rigidly connecting said mold to one of said elements, separated mass means rigidly connected to said second element and having a mass such as to make the entire 45 mass fixed to and including said second element at least substantially equal to that fixed to and including said first element and means for providing a restoring force between said elements sufficient to make the resulting system resonant 50 at the desired oscillation frequency.

45 5. Apparatus for imparting rotational oscillations to a crucible for molten metal comprising, in combination, therewith a stationary base element, means for supporting said crucible upon said base so as to be free to oscillate with re-

5 spect thereto, an electromagnetic system having field and armature elements for producing rotational oscillation energy, one of said elements being mechanically fixed to said crucible supporting means, means for supporting said second element upon said base so as to be free to oscillate with respect thereto and with respect to said first element, a separated mass element mechanically fixed to said second element and of a magnitude sufficient to make the combined 10 mass of the elements connected to it at least substantially equal to the combined mass of the crucible when filled and the elements connected to it and resilient means adapted to provide a restoring force to make the system oscillate at a 15 natural frequency equal to the desired frequency of oscillation.

6. Apparatus for vibrating molten metal at high velocity comprising a resonant vibratory system composed of a single freely vibratable 20 mass element, an elastic element and a stationary second mass element whose mass is substantially infinite relative to the first mass element, said elastic element being fixed at one end to one of said mass elements and at the other end 25 to the other of said mass elements, the first mass element including the molten metal, a container therefor and ancillary elements adapted to move therewith, said elastic element having sufficient elasticity to make the vibratory system resonant 30 at the desired frequency of vibration and means for supplying vibratory energy to vibrate the system at the said resonant frequency.

7. Apparatus for vibrating molten metal at high velocity comprising a resonant vibratory 35 system composed of two freely vibratable independent mass elements and an elastic element fixed at one end to one of said mass elements and at the other end to the other of said mass elements, the first mass element including the 40 molten metal, a container therefor and ancillary elements movable therewith, the second mass element being a compensating mass, said elastic element having sufficient elasticity to make the vibratory system resonant at the desired frequency of vibration and means for supplying vibratory energy to vibrate the system at the said 45 resonant frequency.

8. Apparatus for vibrating molten metal at high velocity comprising a resonant vibratory 50 system composed of a single freely vibratable mass element, an elastic element and a stationary second mass element whose mass is substantially infinite relative to the first mass element, said elastic element being fixed at one end to one of 55 said mass elements and at the other end to the other of said mass elements, the first mass element including the molten metal, a container therefor and ancillary elements adapted to move therewith, said elastic element having sufficient 60 elasticity to make the vibratory system resonant at the desired frequency of vibration and electromagnetic means for supplying vibratory energy to vibrate the system at the said resonant frequency including armature and field elements, one of said 65 elements being fixed to said first mass and the other of said elements being fixed to said second mass, said elements being positioned to cooperate with each other electromagnetically.

9. Apparatus for vibrating molten metal at 70 high velocity comprising a resonant vibratory system composed of two freely vibratable independent mass elements and an elastic element fixed at one end to one of said mass elements and at the other end to the other of said mass 75

- elements, the first mass element including the molten metal, a container therefor and ancillary elements movable therewith, the second mass element being a compensating mass, said elastic element having sufficient elasticity to make the vibratory system resonant at the desired frequency of vibration and electromagnetic means for supplying vibratory energy to vibrate the system at the said resonant frequency including
- 5 10 armature and field elements, one of said elements being fixed to said first mass and the other of said elements being fixed to said second mass, said elements being positioned to cooperate with each other electromagnetically.
- 15 10. Apparatus for vibrating molten metal at high velocity comprising a resonant vibratory system composed of two freely vibratable independent mass elements and an elastic element fixed at one end to one of said mass elements and at the other end to the other of said mass elements, the first mass element including the molten metal, a container therefor and ancillary elements movable therewith, the second mass element being a compensating mass having a total mass substantially equal to the total mass of the
- 20 25

first mass element, said elastic element having sufficient elasticity to make the vibratory system resonant at the desired frequency of vibration and means for supplying vibratory energy to vibrate the system at the said resonant frequency.

11. Apparatus for vertically vibrating a container for molten metal comprising a two-mass resonant vibratory system composed of two freely vibratable masses and an elastic element fixed at one end to one of said mass elements and at the other end to the other of said mass elements, one of said masses including the metal, its container and ancillary elements adapted to move therewith, said elastic element having sufficient elasticity to make the vibratory system resonant at the desired frequency of vibration and resilient means for supporting the said vibratory system, the total mass of the latter and the resilient means forming a second vibratory system, the elasticity of the resilient means being so adjusted that the resonance of said second vibratory system is at a frequency substantially different from the resonant frequency of the first vibratory system.

EDWARD W. SMITH. 25